

1

**3,258,338**  
**PHOTOGRAPHIC MATERIAL CONTAINING**  
**SOFTENING AGENT**

Daniël Aloïs Claeys, Guido Gezellelaan 104, Mortsel-Antwerp, Belgium; Jozef Frans Willems, Sterrenlaan 52, Wilrijk-Antwerp, Belgium; and Marcel Nicolas Vrancken, Ringlaan 31, Berchem-Antwerp, Belgium  
 No Drawing. Filed Dec. 26, 1961, Ser. No. 162,272  
 Claims priority, application Belgium, Dec. 29, 1960, 40,328, Patent 598,619; June 26, 1961, 40,757; Germany, June 27, 1961, G 32,594  
 16 Claims. (Cl. 96—67)

This invention relates to a process for improving the physical properties of a photographic material and more particularly to an improved process for softening gelatin containing layers of such a photographic material.

When using gelatin photographic materials it is important to incorporate softening agents to the gelatin for rendering the gelatin layers made therefrom better resistant to treatments at a low relative humidity. Indeed, gelatin layers or gelatin containing layers without softening agents are very brittle at low degree of relative humidity.

It is known to add to gelatin polyalcohols such as glycerol, lactic acid, substituted phenols monoglycerides of fatty acids or amides such as formanilide as a softening agent.

As compounds improving the elasticity and the flexibility of gelatino silver halide emulsion layers, water-soluble long-chained aliphatic amines containing an amide function, metal soaps of sulfonated castor oil which are insoluble in the photographic processing baths, poly(methoxy alcohols) and aqueous dispersions of poly(ethyl acrylate) are also added.

As softening agents for gelatin it is further known to use compounds with a substituted amide group as described in French patent specification 1,114,721.

Some of these products such as glycerol or other polyalcohols are strongly hygroscopic and thus injure the photographic and physical properties of the layers at rather high relative humidity.

Softening agents for articles made of proteinaceous material are not numerous since the compatibility of the softening agents with the proteinaceous material is mostly insufficient.

In choosing softening agents for gelatin used for photographic purposes, there has moreover to be paid attention to their possible influence on the photographic properties of the materials to be manufactured. In some cases the transparency of the material should not be injured by the addition of softening agents.

The use of phosphoric acid esters such as tributyl phosphate, tricresyl phosphate and triphenyl phosphate as softening agents for articles containing cellulose esters is already known since a long time (Kirk-Othmer, Encyclopedia of Chemical Technology, p. 766).

It has now been found that some organic compounds of phosphonic acid and phosphoric acid are excellent softening agents for articles of proteinaceous materials such as gelatin or casein, and that these softening agents soften layers containing proteinaceous materials if they are added thereto in an amount of at least 3% by weight of the dry proteinaceous material.

The phosphonic acid compounds and phosphoric acid compounds used according to the invention correspond to the following general formula:



2

wherein

Each of  $\text{R}_1$  and  $\text{R}_2$  represents an alkyl radical or an  $\text{R}_4-(\text{O}-\text{alkylene})_n-\text{O}-$  radical, preferably an



radical,

$\text{R}_3$  represents a hydroxyl group, an alkyl radical, an alkoxy radical or an  $\text{R}_4-(\text{O}-\text{alkylene})_n-\text{O}-$  radical, preferably an  $\text{R}_4-(\text{O}-\text{CH}_2-\text{CH}_2)_n-\text{O}-$  radical, wherein  $\text{R}_4$  represents an alkyl radical, an alkaryl radical or an acyl radical,

And  $n$  represents an integer of from 1 to 50.

Mixtures of softening agents according to the above general formula can also be used.

The phosphonic and phosphoric acid compounds used according to this invention can easily be prepared from the corresponding acid chlorides or acid anhydrides by reaction with higher as well as with lower alcohols, with monoalkylene glycol alkylethers or with polyoxoalkylene glycol monoalkyl ethers.

The following compounds and some of their preparations illustrate the present invention. Many of these compounds are commercially available.

**COMPOUND 1.—TRIETHYL ORTHOPHOSPHORIC ACID ESTER**

This compound is marketed as "Triethyl Phosphate" by Albright & Wilson, Ltd., London.

**COMPOUND 2.—TRI-N-BUTYL ORTHOPHOSPHORIC ACID ESTER**

This compound is marketed as "Tri-n-butyl Phosphate" by Albright & Wilson, Ltd., London.

**COMPOUND 3.—TRIETHYL PHOSPHONIC ACID ESTER**

This compound is marketed as "Diethyl ethyl phosphonate" by Virginia-Carolina Chemical Corporation, Richmond, Va., U.S.A.

**COMPOUND 4.—TRI(2-METHOXYETHYLENE) PHOSPHATE**

In a three-necked flask of 5 liter fitted with a stirrer, a thermometer, a condenser, a dropping funnel and the necessary calcium chloride tubes, the following mixture is stirred and cooled till 0° C.:

50 228 g. (3 mol) of ethyleneglycol monomethyl ether  
 237 g. (3 mol) of pyridine  
 1000 c.<sup>3</sup> of anhydrous benzene

60 While the temperature is kept between 0 and 5° C., 154 g. (1 mol) of phosphorus oxychloride are dropwise added in two hours, whereby a precipitate of pyridine hydrochloride is formed. The mixture is still stirred for one hour. Thereupon 500 cm.<sup>3</sup> of water are added and the formed benzene layer is separated. The benzene is distilled on a water-bath under a fractionating column with the air of the reduced pressure of a water-jet pump in order to collect the main fraction of the residue having a boiling range of 202–218° C. at 15 mm. Hg of pressure. After renewed distillation by means of an oil vacuum pump, the desired fraction is obtained which distills between 158 and 160° C. at about 1 mm. Hg of pressure.

## 3

## COMPOUND 5.—TRI(2-ETHOXYETHYLENE) PHOSPHATE

In a three-necked flask of 5 liter fitted with a stirrer, a thermometer, a condenser, a dropping funnel and the necessary calcium chloride tubes, the following mixture is stirred and cooled till 0° C.:

270 g. (3 mol) of ethylene glycol monoethylether  
237 g. (3 mol) of pyridine  
1000 cm.<sup>3</sup> of anhydrous benzene

While the temperature is kept between 0 and 5° C., 154 g. (1 mol) of phosphorus oxychloride are dropwise added in two hours, whereby a precipitate of pyridine hydrochloride is formed. The mixture is still stirred for one hour. Thereupon 500 cm.<sup>3</sup> of water are added and the formed benzene layer is separated. The benzene is distilled on a water-bath under a fractionating column with the aid of the reduced pressure of a water-jet pump. The residue is first distilled at about 1 mm. Hg of pressure without fractionation and thereupon fractionated at the same pressure in order to collect the fraction with boiling range of 150–158° C.

Yield: 78 g.

## COMPOUND 6.—TRI(DIETHYLENE GLYCOL MONOMETHYL ETHER) PHOSPHATE

In a three-necked flask of 3 liter fitted with a stirrer, a thermometer, a condenser, a dropping funnel and the necessary calcium chloride tubes the following mixture is stirred and cooled till 0° C.:

25 252 g. (2.1 mol) of diethylene glycol monomethyl ether  
237 g. (3 mol) of pyridine  
1000 cm.<sup>3</sup> of anhydrous benzene

While the temperature is kept between 0° and 5° C., 154 g. (1 mol) of phosphorus oxychloride are dropwise added in two hours, whereby a precipitate of pyridine hydrochloride is formed. The mixture is still stirred for one hour and thereupon 500 cm.<sup>3</sup> of water are added. The benzene layer is separated and the benzene is distilled on a water-bath under a fractionating column with the aid of the reduced pressure of a water-jet pump. The residue is distilled at about 1 mm. Hg of pressure in order to collect the main fraction with boiling range of 150–158° C.

Yield: 78 g.

## COMPOUND 7.—TRI(DIETHYLENE GLYCOL MONOETHYL ETHER) PHOSPHATE

In a three-necked flask of 3 liter, fitted with a stirrer, a thermometer, a condenser, a dropping funnel and the necessary calcium chloride tubes, the following mixture is stirred and cooled till 0° C.:

50 402 g. (3 mol) of diethylene glycol monoethyl ether  
237 g. (3 mol) of pyridine  
1000 cm.<sup>3</sup> of anhydrous benzene

While the temperature is kept between 0° and 5° C., 154 g. (1 mol) of phosphorus oxychloride are dropwise added in two hours. The mixture is still stirred for 1 hr. The formed pyridine hydrochloride is sucked off and washed with anhydrous benzene. The benzene filtrate is evaporated with the aid of a water-jet vacuum pump whereby a pale yellow oil is left. Then the carbitol residue is removed by extraction with hexane, whereupon 80 cm.<sup>3</sup> of 5 N sodium hydroxide are added. The formed mixture consisting of two layers is first heated for 30 min., then cooled and finally extracted with ether for 8 hours. The obtained ether-extract is dried over anhydrous sodium sulfate and after drying the ether is distilled. The residue is then kept for 2 hours on a water-bath in the reduced pressure formed by a water-jet pump in order to eliminate the remained traces of pyridine, if still present.

Yield: 150 g.

## 4

## COMPOUND 8

The softening agent with the following composition:



is prepared as follows:

15     A mixture consisting of 32.2 g. of tridecyloxy triethylene glycol, 8 g. of pyridine, 5.1 g. of phosphorus oxychloride and 50 cm.<sup>3</sup> of benzene is refluxed for 1 hr. After cooling, the formed precipitate of pyridine hydrochloride is sucked off. In order to remove completely the pyridine under the form of its hydrochloride, hydrochloric gas is led through the solution and the formed hydrochloride is once again filtered off. Then the benzene is distilled under reduced pressure.

## COMPOUND 9

The softening agent with the following composition



is prepared as follows:

35     A mixture consisting of 125 g. of tridecyloxy penta-decaethylene glycol, 4 g. of pyridine, 25 g. of phosphorus oxychloride and 50 cm.<sup>3</sup> of benzene is refluxed for 1 hr. After cooling, the formed pyridine hydrochloride is filtered off and hydrochloric gas is led through the benzene solution. After filtration, the benzene solution is stirred and boiled with 10 cm.<sup>3</sup> of water and then evaporated to dryness.

## COMPOUND 10

The softening agent with the following composition



is prepared as follows:

55     A mixture consisting of 20 g. of the condensation product of 5 mol of ethylene oxide and 1 mol of stearic acid, 50 cm.<sup>3</sup> of anhydrous ether and 0.95 g. of dry phosphorus pentoxide is refluxed for 2 hr. Thereupon the ether is distilled.

## COMPOUND 11

The softening agent with the following composition



70     is prepared as follows:

75     A mixture consisting of 20 g. of the condensation product of 10 mol of ethylene oxide and 1 mol of stearic acid, 50 cm.<sup>3</sup> of anhydrous ether and 0.66 g. of dry phosphorus pentoxide is refluxed for 2 hr. Thereupon the ether is distilled.

## 5

## COMPOUND 12

The softening agent with the following composition:



is prepared as follows:

A mixture consisting of 20 g. of the condensation product of 15 mol of ethylene oxide and 1 mol of stearic acid, 50 cm.<sup>3</sup> of anhydrous ether and 0.51 g. of anhydrous phosphorus pentoxide is refluxed for 2 hr. Thereupon the ether is distilled.

## COMPOUND 13

The softening agent with the following composition



is prepared as follows:

A mixture consisting of 20 g. of the condensation product of 50 mol of ethylene oxide and 1 mol of stearic acid, 50 cm.<sup>3</sup> of anhydrous ether and 0.20 g. of dry phosphorous pentoxide is refluxed for 2 hr. Thereupon the ether is distilled.

## COMPOUND 14

The softening agent with the following composition



is prepared as follows:

A mixture consisting of 16 g. of the condensation product of 6 mol of ethylene oxide and 1 mol of nonyl phenol, 50 cm.<sup>3</sup> of anhydrous ether and 1.2 g. of dry phosphorous pentoxide is refluxed for 2 hr. Thereupon the ether is distilled.

## COMPOUND 15

The softening agent with the following composition



## 6

A mixture consisting of 20 g. of the condensation product of 15 mol of ethylene oxide, 1 mol of nonyl phenol, 0.8 g. of dry phosphorous pentoxide and 50 cm.<sup>3</sup> of anhydrous ether is refluxed for 2 hr. Thereupon the ether is distilled.

## COMPOUND 16

The softening agent with the following composition



is prepared as follows:

A mixture consisting of 20 g. of the condensation product of 30 mol of ethylene oxide and 1 mol of nonyl phenol, 0.5 g. of dry phosphorous pentoxide and 50 cm.<sup>3</sup> of anhydrous ether is refluxed for 2 hr. Thereupon the ether is distilled.

## COMPOUND 17

The softening agent with the general formula



is marketed under the trade-name Hostaphat KL 240 by Farbwerke Hoechst A.G., Frankfurt am Main Hochst, Germany.

## COMPOUND 18

The softening agent with the general formula



is marketed under the trade-name Hostaphat KO 280 by Farbwerke Hoechst A.G., Frankfurt am Main Hochst, Germany.

The softening agents, according to the present invention can be used in various compositions of matter.

They are especially suited for being incorporated in gelatin containing layers which form part of a photographic material.

The phosphonic and phosphoric acid compounds according to the invention can favorably be applied in a photographic silver halide emulsion layer or in another gelatin containing layer of a light sensitive photographic material such as an antihalation layer or other backing layer or supercoat on the emulsion layer as well as in gelatin containing layers of an image-receiving material for the manufacture of images according to the silver complex diffusion transfer process described in U.S. patent specification 2,352,014. These softening agents can also favorably be used in the gelatin layer of the so-called blank film described in French patent specification 1,265,552. These layers may comprise compounds such as colour couplers, chemical or optical sensitizers, anti-fogging agents, optical brightening agents, wetting agents, development accelerators and matting agents, and can be cast upon paper, glass plates or films e.g. of cellulose esters, polyesters, polystyrene, etc.

The softening agents according to this invention have also a good antistatic effect. This effect is strongly pronounced when the softening agent is incorporated into a layer which is in the outer side of the photographic material such as a backing layer.

Not all softening agents according to the present invention are equally well suited for being applied in light-sensitive silver halide emulsion layers. Softening agents with a molecular weight of more than 1500 and having more than 20 oxyalkylene groups in their structure, when applied in the light-sensitive silver halide emulsion layer in an amount as small as possible in order to obtain a practically usable softening effect give already rise to formation of fog. Such softening agents, however, can be used in another layer than the silver halide emulsion layer of a photographic material.

The amount of softening agent which can be used depends on the desired improvement of the flexibility of the layers wherein they are incorporated. Preferably these compounds are used in an amount of 10% to 30% based on the weight of dry proteinaceous material.

The phosphonic and phosphoric acid compounds according to this invention are preferably added before coating the gelatin solution. In order to obtain a good dispersion some of these compounds with no more than 5 alkylene oxide groups, are preferably emulsified in the gelatin solution by means of emulsifying agents.

The most suitable emulsifying agents are the anion-active wetting agents such as sodium salts of alkylsulfonic acids e.g. sodium tetradecylsulfate and the sodium salt of the condensation product of oleic acid and methyltaurine of the formula



In order to compare the increased flexibility of gelatin containing layers containing softening agents according to this invention with the flexibility of usually treated gelatin layers folding tests were carried out with a M.I.T. fold tester. By means of this apparatus the number of folds until breaking can be determined.

The following examples illustrate the present invention.

#### Example 1

The equal parts of a 10% aqueous solution of gelatin at pH 7 to 8, 20% of the compounds identified in the following table, based on the weight of the dry gelatin, are added. After thoroughly mixing the gelatin solutions are applied onto glass-plates which are treated previously in such a way that after drying, the gelatin layers can easily be stripped off.

After solidifying and drying at room-temperature, the gelatin layers with a thickness of about 150  $\mu$  are stripped off and cut into strips with a width of 15 mm. Thereupon the number of folds until breaking are determined with a M.I.T. fold tester at 30% relative humidity and 20° C.

The following results are obtained:

| Softening agent: | Number of folds until breaking | 55 |
|------------------|--------------------------------|----|
| None             | 6                              |    |
| Glycerol         | 18                             |    |
| Compound 1       | 64                             |    |
| Compound 2       | 35                             |    |
| Compound 3       | 12                             |    |
| Compound 4       | 32                             |    |
| Compound 5       | 77                             |    |
| Compound 6       | 38                             |    |
| Compound 7       | 40                             |    |
| Compound 8       | 286                            | 65 |
| Compound 9       | 35                             |    |
| Compound 10      | 117                            |    |
| Compound 11      | 22                             |    |
| Compound 12      | 15                             |    |
| Compound 13      | 26                             | 70 |
| Compound 14      | 46                             |    |
| Compound 15      | 22                             |    |
| Compound 16      | 36                             |    |
| Compound 17      | 119                            |    |
| Compound 18      | 85                             | 75 |

The compounds 1, 3, 4, 5, 6 and 7 were added to the gelatin solution by means of the emulsifying agent Tergitol 4 (trade-name for a 25% aqueous solution of sodium tetradecyl sulfate marketed by Union Carbide and Carbon, New York, N.Y., U.S.A.).

#### Example 2

160 cm.<sup>3</sup> of a 10% alcoholic solution of compound 8 are added to 1 kg. of a light-sensitive silver halide emulsion comprising 80 g. of gelatin. This emulsion is cast onto a cellulose triacetate support and dried.

The number of folds until breaking of the emulsion strips determined at 30% relative humidity and 20° C. with a M.I.T. fold tester amounts to 20. A similar emulsion strip without softening breaks at the fourth fold.

#### Example 3

##### LAYER A

To 1 liter of a 8% aqueous solution of gelatin containing an anti-halation dyestuff, 150 cm.<sup>3</sup> of a 10% alcoholic solution of the softening agent described as compound 8 in Example 1 are added. The solution is applied onto a cellulose triacetate support and dried.

##### LAYER B

To 1 liter of a 8% aqueous solution of gelatin containing manganese dioxide, 150 cm.<sup>3</sup> of a 10% alcoholic solution of the softening agent described as compound 8 in Example 1 are added. The solution is applied onto a cellulose triacetate support and dried.

The flexibility of both anti-halation layers is tested with a M.I.T. fold tester at 20° C. and at 30% and 36% relative humidity. Two layers C and D, prepared in the same way as the layers A and B but containing no softening agent, are also tested. The following results are obtained:

| Anti-halation layer | Number of folds until breaking |          |
|---------------------|--------------------------------|----------|
|                     | 30% R.H.                       | 36% R.H. |
| A                   | 21                             | 40       |
| B                   | 26                             | 38       |
| C                   | 12                             | 20       |
| D                   | 14                             | 19       |

We claim:

1. Photographic material comprising a support and at least one gelatin layer containing a compound of the formula:



each of R<sub>1</sub> and R<sub>2</sub> (equal or different) represents an alkyl radical or a R<sub>4</sub>—(O-alkylene)<sub>n</sub>— radical, R<sub>3</sub> represents a hydroxyl group, an alkyl radical, an alkoxy radical, or a R<sub>4</sub>—(O-alkylene)<sub>n</sub>—O— radical wherein R<sub>4</sub> represents an alkyl radical, an alkaryl radical or an acyl radical, and n represents an integer of from 1 to 50,

said compound being present in a quantity of at least 3% by weight of the gelatin.

2. Photographic material according to claim 1 wherein said one gelatin layer is a gelatino silver halide emulsion layer, said compound being present in an amount equal to at least 3% by weight of the gelatin in said layer.

3. Photographic material according to claim 1 comprising at least one gelatino silver halide emulsion layer and at least one other gelatin layer free of silver halide emulsion, and wherein each of said gelatino emulsion layer and said other gelatin layer contain a compound corresponding to the formula of claim 1 in an amount equal to at least 3% by weight of the gelatin therein.

4. The photographic material of claim 1 wherein said layer contains a mixture of 80% of a compound of the formula



and 20% of a compound of the formula



5. The photographic material of claim 1 wherein said layer contains a mixture of 90% of a compound of the formula



and 10% of a compound of the formula



6. The photographic material of claim 1 wherein said layer contains a compound of the formula



7. The photographic material of claim 1 wherein said layer contains a compound of the formula



8. Sheet material comprising a support and at least one gelatin layer containing a compound of the formula:



wherein

R<sub>1</sub> and R<sub>2</sub> each represents an R<sub>4</sub>—(O-alkylene)<sub>n</sub>— radical or an R<sub>4</sub>—CO—(O-alkylene)<sub>n</sub>— radical

R<sub>3</sub> represents a hydroxyl group, an



radical or an R<sub>4</sub>—CO—(O-alkylene)<sub>n</sub>—O— radical in which formula R<sub>4</sub> represents a hydrocarbon radical, and n represents a positive number from 1 to 50.

9. Sheet metal according to claim 8, wherein said compound is present in an amount equal to at least 3% by weight of the gelatin in said layer.

10. Sheet material according to claim 8, wherein n represents a positive number of 3 to 8.

11. Sheet material according to claim 10, wherein the

hydrocarbon radical is a saturated or unsaturated, aliphatic hydrocarbon radical containing from 10 to 20 carbon atoms.

12. Sheet material according to claim 11, wherein the alkylene group is an ethylene group and wherein the saturated or unsaturated aliphatic hydrocarbon radical has 12 to 17 carbon atoms.

13. The sheet material of claim 8, wherein said layer contains a mixture of 80% of a compound of the formula



and 20% of a compound of the formula



14. The sheet material of Claim 8, wherein said layer contains a mixture of 90% of a compound of the formula



and 10% of a compound of the formula



15. The sheet material of claim 8, wherein said layer contains a compound of the formula



16. The sheet material of claim 8, wherein said layer contains a compound of the formula



#### References Cited by the Examiner

##### UNITED STATES PATENTS

|           |         |               |         |
|-----------|---------|---------------|---------|
| 2,887,381 | 5/1959  | Levy          | 96—94   |
| 2,940,854 | 6/1960  | Gray          | 96—94   |
| 2,950,980 | 8/1960  | Hirsch        | 106—125 |
| 2,958,605 | 11/1960 | Leiner et al. | 106—125 |
| 3,058,941 | 10/1962 | Birum         | 106—125 |

##### OTHER REFERENCES

Buttrey, D. N., Plasticizers, London, Cleaver-Hume Press Ltd., 1957, pp. 35, 36.

NORMAN G. TORCHIN, Primary Examiner.

ALEXANDER D. RICCI, Examiner.

C. E. DAVIS, Assistant Examiner.

UNITED STATES PATENT OFFICE  
CERTIFICATE OF CORRECTION

Patent No. 3,258,338

June 28, 1966

Daniël Aloïs Claeys et al.

It is hereby certified that error appears in the above numbered patent requiring correction and that the said Letters Patent should read as corrected below.

In the grant, line 4, after "Belgium," insert -- assignors to Gevaert Photo-Producten N.V., of Mortsel, Belgium, a company of Belgium --; lines 13 and 14, for "Daniël Aloïs Claeys, Jozef Frans Willems, and Marcel Nicolas Vrancken, their heirs" read -- Gevaert Photo-Producten N.V., its successors --; in the heading to the printed specification, lines 4 to 7, for "Daniël Aloïs Claeys, Guido Gezellelaan 104, Mortsel-Antwerp, Belgium; Jozef Frans Willems, Sterrenlaan 52, Wilrijk-Antwerp, Belgium; and Marcel Nicolas Vrancken, Ringlaan 31, Berchem-Antwerp, Belgium" read -- Daniël Aloïs Claeys, Mortsel-Antwerp, Belgium; Jozef Frans Willems, Wilrijk-Antwerp, Belgium; and Marcel Nicolas Vrancken, Berchem-Antwerp, Belgium, assignors to Gevaert Photo-Producten N.V., Mortsel, Belgium, a company of Belgium --.

Signed and sealed this 25th day of March 1969.

(SEAL)

Attest:

EDWARD M. FLETCHER, JR.  
Attesting Officer

EDWARD J. BRENNER  
Commissioner of Patents